

# United States Patent [19]

[ 19 ]

Mitchell

[11] 3,723,347

Mar. 27, 1973

- [54] **CORROSION INHIBITION COMPOSITIONS CONTAINING SUBSTITUTED DIAMINE PHOSPHONATES AND PROCESSES FOR USING THE SAME**

[75] Inventor: **Robert S. Mitchell, Webster Groves, Mo.**

[73] Assignee: **Monsanto Company, St. Louis, Mo.**

[22] Filed: **May 17, 1972**

[21] Appl. No.: **254,008**

[52] U.S. Cl. .... **252/389 A, 21/2.7 A, 106/14, 210/58, 252/181, 252/387, 252/389 R, 252/390, 260/502.5**

[51] Int. Cl. .... **C23f 11/16**

[58] Field of Search .... **252/389 A, 389 R, 387, 181, 252/390; 21/2.7, 2.5; 260/502.5; 106/14; 210/58**

3,431,217 3/1969 Hwa ..... 252/387  
 3,483,133 12/1969 Hatch ..... 252/389 A

*Primary Examiner*—Leon D. Rosdol  
*Assistant Examiner*—Irwin Gluck  
*Attorney*—James J. Mullen et al.

[57] **ABSTRACT**

Substituted diamine phosphonates of the general formula

$$\begin{array}{c}
 \text{O} \quad \text{X} \\
 \text{R}_1\text{O}-\text{P} \text{---} \text{C} \text{---} \text{N}-\text{Z}-\text{N}[(\text{R}_3\text{O})_n(\text{R}_4\text{OH})]_2 \\
 | \quad \quad | \\
 \text{O} \quad \text{Y} \\
 \text{R}_1\text{O}-\text{P} \text{---} \text{C} \text{---} \text{N}-\text{Z}-\text{N}[(\text{R}_3\text{O})_n(\text{R}_4\text{OH})]_2
 \end{array}$$

[56] References Cited

UNITED STATES PATENTS

- |           |         |                       |           |
|-----------|---------|-----------------------|-----------|
| 2,961,311 | 11/1960 | Bersworth et al. .... | 260/502.5 |
| 3,160,632 | 12/1964 | Toy et al. ....       | 260/502.5 |
| 3,298,956 | 1/1967  | Irani et al. ....     | 260/502.5 |
| 3,336,221 | 8/1967  | Ralston ....          | 260/502.5 |
| 3,395,113 | 7/1968  | Irani et al. ....     | 260/502.5 |

*Primary Examiner*—Leon D. Rosdol  
*Assistant Examiner*—Irwin Gluck

*Assistant Examiner*—H. Will Gluck  
*Attorney*—James J. Mullen et al

*Attorney*—James J. Mullen et al.

[57]

## ABSTRACT

## Substituted diamine phosphonates of the general formula



wherein  $R_1$ ,  $R_2$ ,  $R_3$ ,  $R_4$ ,  $X$ ,  $Y$  and  $Z$  are hereinafter defined and  $n$  is 0-10, alone or in combination with zinc, dichromates, certain thiols, 1,2,3-triazoles, silicates, inorganic phosphates, molybdates, tannins, lignins, lignin sulfonates, certain calcium and magnesium salts and mixtures thereof, are disclosed as inhibiting the corrosion of metals by oxygen-bearing waters.

**34 Claims, No Drawings**

**CORROSION INHIBITION COMPOSITIONS  
CONTAINING SUBSTITUTED DIAMINE  
PHOSPHONATES AND PROCESSES FOR USING  
THE SAME**

The present invention relates to corrosion inhibiting compositions and to methods of inhibiting the corrosion of metal surfaces in contact with an aqueous medium of a corrosive nature. More particularly, this invention relates to methods of inhibiting the corrosion of metal surfaces by utilizing in the corrosive aqueous medium certain substituted diamines either alone or in combination with a water-soluble zinc salt, a dichromate, certain thiols, 1,2,3-triazoles, silicates, inorganic phosphates, molybdates, tannins, lignins, lignin sulfonates, certain calcium and magnesium salts and mixtures thereof.

The present invention has special utility in the prevention of the corrosion of metals which are in contact with circulating water, that is, water which is moving through condensers, engine jackets, cooling towers, evaporators or distribution systems, however, it can be used to prevent the corrosion of metal surfaces in other aqueous corrosive media. This invention is especially valuable in inhibiting the corrosion of ferrous metals including iron and steel (also galvanized steel) and non-ferrous metals including copper and its alloys, aluminum and its alloys and brass. These metals are generally used in circulating water systems.

The major corrosive ingredients of aqueous cooling systems are primarily dissolved oxygen and inorganic salts, such as the carbonate, bicarbonate, chloride and/or sulfate salts of calcium, magnesium and/or sodium.

It is, therefore, a primary object of this invention to provide new corrosion inhibiting methods.

It is another object of this invention to provide new corrosion inhibiting methods for ferrous metals including iron and steel and non-ferrous metals including copper and brass.

It is another object of this invention to provide new and corrosion inhibiting methods for ferrous metals including iron and steel and non-ferrous metals including copper and brass in contact with an aqueous corrosive medium.

It is another object of this invention to provide new corrosion inhibiting methods for ferrous metals including iron and steel and non-ferrous metals including copper and brass in contact with cooling waters.

Other advantages and objects of the present invention will be apparent from the following discussion and appended claims.

It has been found that certain substituted diamines corresponding to the following formula



unexpectedly function as corrosion inhibitors when used alone or in combination with zinc, dichromate, certain thiols and 1,2,3-triazoles, silicates, inorganic phosphates, molybdates, tannins, lignins, lignin sul-

fonates, certain calcium and magnesium salts and mixtures thereof in aqueous or water systems containing metals or in contact with metals.

In Formula I above, R<sub>1</sub> and R<sub>2</sub> can be alike or unlike and are from the group metal ion or hydrogen or any cation which will yield sufficient solubility for the desired end-use. The aforementioned cations are from the group of metals alkali metals such as sodium, lithium, potassium, alkaline earth metals such as calcium and magnesium, aluminum, zinc, cadmium, manganese, nickel, cobalt, cerium, lead, tin, iron, chromium, and mercury. Also included are amines such as ammonium ions and alkyl ammonium ions. In particular, those alkyl ammonium ions derived from amines having a low molecular weight, such as below about 300, and more particularly the alkyl amines, alkylene amines, and alkanol amines containing not more than two amine groups, such as ethyl amine, diethyl amine, propyl amine, propylene diamine, hexyl amine, 2-ethylhexylamine, N-butylethanol amine, triethanol amine, and the like, are the preferred amines. It is within the scope of the present invention to include amines, such as those described in U.S. Pat. Nos. 3,613,788 and 3,619,427 (which are incorporated herein by reference), in order to provide the amine salts of the aforesaid substituted diamines (Formula I). It is to be understood that the preferred metal ions are those which render the compound a water-soluble salt, e.g., sodium, in concentrations sufficient for the desired applications.

In Formula I, it is to be understood that this includes salts, partial salts, acid and partial acids.

In Formula I above, R<sub>3</sub> and R<sub>4</sub> are alike or unlike and are each independently an alkylene group containing from two to five, preferably two to three carbon atoms. Examples of such alkylene groups include, without limitation, ethylene, propylene, butylene and the like.

In Formula I, and partial Formula II above, X and Y are each alike or unlike and are from the group hydrogen and organic radicals such as alkyl containing less than 40, preferably one to four, carbon atoms. It is to be understood that organic radicals such as other aliphatic groups and also aromatic groups are included herein. X and Y are preferably hydrogen.

In Formula I, Z is a hydrocarbon group containing from two to 15 carbon atoms and includes (a) normal or straight chain carbon groups, e.g., (CH<sub>2</sub>)<sub>2</sub> to (CH<sub>2</sub>)<sub>15</sub>, (b) branched chain carbon groups, e.g., —CH<sub>2</sub>CH<sub>2</sub>CH<sub>2</sub>—, and (c) cyclic carbon groups, e.g.,



60 In Formula I, n has a value of from 0 through 10 (preferably 0-3). It is to be understood that all of the compounds falling within the above Formula I and as heretofore defined are generically described herein as "substituted diamines" or SDA. In other words, then, the acids, salts and physical and chemical mixtures thereof are all generically described herein as "substituted diamines" or "SDA."

Illustrative (but without limitation) of some of the present invention SDA corrosion inhibitors are shown below:

(I)



| Compound No. | R <sub>1</sub> | R <sub>2</sub>  | R <sub>3</sub>                | R <sub>4</sub>                | X               | Y | n                                 | Z                               |
|--------------|----------------|-----------------|-------------------------------|-------------------------------|-----------------|---|-----------------------------------|---------------------------------|
| 1            | H              | H               |                               | C <sub>2</sub> H <sub>4</sub> | H               | H | 0                                 | (CH <sub>2</sub> ) <sub>3</sub> |
| 2            | "              | K               |                               | "                             | "               | " | 0                                 | "                               |
| 3            | "              | Na              |                               | "                             | "               | " | 0                                 | "                               |
| 4            | "              | ZN              |                               | "                             | "               | " | 0                                 | "                               |
| 5            | "              | NH <sub>4</sub> |                               | "                             | "               | " | 0                                 | "                               |
| 6            | "              | H               | C <sub>2</sub> H <sub>4</sub> | "                             | "               | " | 1                                 | "                               |
| 7            | "              | "               | "                             | "                             | "               | " | 5                                 | "                               |
| 8            | "              | "               | "                             | "                             | "               | " | 10                                | "                               |
| 9            | "              | "               | C <sub>3</sub> H <sub>6</sub> | C <sub>3</sub> H <sub>6</sub> | "               | " | 1                                 | "                               |
| 10           | "              | Na              | "                             | "                             | "               | " | 1                                 | "                               |
| 11           | "              | H               | "                             | "                             | "               | " | 5                                 | "                               |
| 12           | "              | "               | C <sub>2</sub> H <sub>4</sub> | "                             | "               | " | 1                                 | "                               |
| 13           | "              | "               | "                             | "                             | "               | " | 5                                 | "                               |
| 14           | Na             | "               | "                             | C <sub>2</sub> H <sub>4</sub> | "               | " | 1                                 | "                               |
| 15           | H              | K               | "                             | "                             | "               | " | 3                                 | "                               |
| 16           | "              | H               | "                             | "                             | CH <sub>3</sub> | " | 0                                 | "                               |
| 17           | "              | "               | "                             | "                             | CH <sub>3</sub> | " | 0                                 | "                               |
| 18           | "              | "               | "                             | C <sub>3</sub> H <sub>6</sub> | H               | H | 0                                 | "                               |
| 19           | "              | "               | "                             | C <sub>2</sub> H <sub>4</sub> | "               | " | 0 (CH <sub>2</sub> ) <sub>2</sub> | 30                              |
| 20           | "              | "               | "                             | "                             | "               | " | 0 (CH <sub>2</sub> ) <sub>4</sub> |                                 |
| 21           | "              | "               | "                             | "                             | "               | " | 0 (CH <sub>2</sub> ) <sub>5</sub> |                                 |
| 22           | "              | "               | "                             | "                             | "               | " | 0 (CH <sub>2</sub> ) <sub>6</sub> |                                 |
| 23           | "              | "               | "                             | "                             | "               | " | 0 C <sub>8</sub> H <sub>10</sub>  |                                 |
| 24           | "              | "               | "                             | "                             | "               | " | 0 C <sub>8</sub> H <sub>14</sub>  |                                 |

The SDA falling within the foregoing Formula I are prepared according to the disclosure set forth in my copending patent application Ser. No. 254,247 filed May 17, 1972 and filed concurrently herewith and which is incorporated herein by reference.

It has been found that to effectively inhibit corrosion, at least 3 parts per million, preferably from about 10 parts per million (ppm) to about 500 parts per million, more preferably from about 10 parts per million to about 150 parts per million, of the SDA should be utilized in the corrosive medium. It is to be understood that greater than 500 ppm of SDA can be utilized where one so desires as long as the desired end result is substantially achieved or these higher amounts are not detrimental to the water system. Amounts as low as 1 ppm are found to be effective.

The SDA corrosion inhibitors of the present invention are effective in both an acidic or basic corrosive media. The pH can range from about 4 to about 12. For example, compound No. 1, heretofore set forth, when used in amounts from about 3 parts per million to about 100 parts per million is an effective corrosion inhibitor in a corrosive medium where the pH is from about 4 to about 12.

In conjunction with the utilization of the SDA per se as corrosion inhibitors, it has also been found that there exists a cooperative effect on corrosion inhibition between the SDA and the zinc ion; that is, the use of the SDA with the zinc ion more effectively inhibits corrosion than does an equal concentration of the SDA or the zinc ion alone. (The zinc ion is used in the same

concentration as the SDA, e.g., a suitable corrosion inhibitor may consist of 50 ppm of zinc ion plus 50 ppm of said SDA.) It is to be understood, then, that the present invention also encompasses a corrosion inhibition compositions containing a mixture of the SDA and a zinc-containing material (i.e., a water-soluble zinc salt) which is capable of forming the zinc ion in an aqueous solution.

Illustrative examples of the zinc-containing material (water-soluble zinc salt) which are set forth for exemplary purposes only and hence non-restrictive, include zinc acetate, zinc bromate, zinc benzoate, zinc borate, zinc bromide, zinc butyrate, zinc caproate, zinc carbonate, zinc chlorate, zinc chloride, zinc citrate, zinc fluoride, zinc fluosilicate, zinc formate, zinc hydroxide, zinc d-lactate, zinc laurate, zinc permanganate, zinc nitrate, zinc hypophosphite, zinc salicylate, zinc sulfate and zinc sulfite. The preferred water-soluble zinc salt is zinc sulfate. It is to be understood that it is within the scope of the present invention that the zinc ion can be supplied in part or wholly by using the zinc salt of the acid form of the SDA.

The SDA and the zinc containing material, which is, in essence, a water-soluble zinc salt, may be mixed as a dry composition and can be fed into a water system containing the metals heretofore described to be protected. Such a composition having a maximum cooperative effect between the SDA and the zinc ion containing material comprises from about 10 percent to about 80 percent by weight of the water-soluble zinc salt and from about 20 percent to about 90 percent by weight of the SDA, all weights being predicated upon the total weight of the mixture. Preferably the weight of the composition comprises from about 20 percent to about 60 percent by weight of the water-soluble zinc salt and from about 40 percent to about 80 percent by weight of the SDA.

a combination of about 3 to 100 ppm A combination the SDA and about 2 to about 100 ppm zinc ion will inhibit corrosion in most water systems; the most preferred concentration range is about 5 to 25 ppm SDA and about 5 to 25 ppm zinc ion. It is to be understood, however, that those concentrations are not in any manner meant to limit the scope of the present invention.

It has also been found that a cooperative effect exists between the SDA and chromate or dichromate. Because chromate and dichromate are each readily converted into the other by a change in pH, it is understood that both will be simultaneously present at most pH's, even though only one is mentioned.

Corrosion in most water systems may be inhibited by adding from about 1 to about 100 ppm of SDA and from about 1 to about 100 ppm of the chromate or dichromate; preferably from about 5 to 25 ppm SDA and from about 5 to 25 ppm chromate or dichromate is added. It is to be understood that larger amounts or smaller amounts of each material can be utilized if one so desires.

Suitable chromates for use in the composition and process of this invention include, for exemplary purposes only, sodium dichromate dihydrate, anhydrous sodium chromate, sodium chromate tetrahydrate, sodium chromate hexahydrate, sodium chromate decahydrate, potassium dichromate, potassium chro-

mate, ammonium dichromate, and chromic acid. In other words, the chromium compound used is any water-soluble hexavalent compound of chromium and is preferably an alkali metal chromate or dichromate heretofore described.

In most cases, an effective corrosion inhibition composition contains a mixture of from about 1 percent to about 60 percent and preferably from about 10 percent to about 40 percent, of the water-soluble inorganic chromate, based on the combined weight of the chromate and SDA. The use of chromates per se is further described in U.S. Pat. No. 3,431,217 and the publications cited in this patent, all of which are incorporated herein by reference.

It has also been found that compositions of the SDA, zinc ion, and chromate or dichromate are useful in inhibiting the corrosion of metals. The inhibiting action of zinc (supplied in the form of a water-soluble zinc salt heretofore mentioned) and dichromate compositions has been shown in U.S. Pat. No. 3,022,133, which is incorporated herein by reference. Thus, all three components of this composition are cooperatively effective. The coaction of zinc and dichromate illustrated in U.S. Pat. No. 3,022,133 remains unaffected in the presence of the SDA and the other ingredients of the inhibitor compositions mentioned herein. In other words, then, it is within the scope of the present invention to provide a corrosion inhibiting composition containing the SDA, a water-soluble zinc salt and a chromate and/or dichromate.

Especially useful combinations of SDA, chromate and zinc exist in the range of from about 1 to about 100 ppm of SDA, from about 1/2 to about 50 ppm of the chromate or dichromate, and from about 1/2 to 50 ppm of the zinc ion. The preferred range is from about 2 to 30 ppm SDA, and from about 1 to 15 ppm chromate or dichromate, and from about 1 to about 15 ppm zinc ion.

Where the water systems are in contact with various metals such as steel, copper per se or copper-containing metals, it is desirable to use, along with the SDA (either alone or in combination with the zinc ion and/or dichromate or chromate), a 1,2,3-thiazole or a thiol of a thiazole, an oxazole, or an imidazole as described respectively in U.S. Pat. Nos. 2,941,953; 2,742,369; and 3,483,133; all of which patents are incorporated herein by reference. These azoles are referred to herein as thiols and 1,2,3-thiazoles. These thiols and 1,2,3-thiazoles are found effective in inhibiting the attack of the SDA on copper.

The preferred 1,2,3-triazole is 1,2,3-benzotriazole of the formula



The preferred thiols of a thiazole, an oxazole, or an imidazole are 2-mercaptopthiazole



2-mercaptopbenzothiazole



2-mercaptopbenzoxazole



15 and 2-mercaptopbenzimidazole



The amounts of thiol or 1,2,3-thiazole used will depend upon the particular water system. Where the water system containing copper is an open or once through system from about 3 to about 100 ppm SDA, about 0.05 to 5 ppm thiol or 1,2,3-triazole, and up to about 100 ppm zinc ion are generally satisfactory concentrations; preferably the concentrations are about 5 to 25 ppm SDA, about 0.5 to 2 ppm triazole or thiol, and about 5 to 25 ppm zinc ion.

A dry composition may be made which may be fed into the water system containing copper. Such a composition would consist of about 20% to 90% by weight, based on the total weight of said composition, SDA; about 1% to 10% by weight thiol or 1,2,3-triazole, and up to about 79% by weight soluble zinc salt; preferably, it would consist of about 38% to 90% by weight SDA, about 2% to 10% by weight thiol or 1,2,3-triazole, and up to about 60% by weight soluble zinc salt.

It is within the scope of the present invention that the corrosion inhibitors (SDA) of this invention may be used in conjunction with other materials (water treating chemicals); in some instances, there can be a cooperative effect therebetween. The following is a list of these materials and publications wherein such materials are utilized in a similar fashion in conjunction with corrosion inhibition.

1. Water-soluble polycarboxylic acids from the group adipic, succinic, azelaic, suberic, sebacic, pimelic, and glutoric acids and hydroxypolycarboxylic acids having from four to 10 carbon atoms and at least 2 carboxylic acids or an alkali metal or ammonium salt thereof—note British Pat. No. 1,230,172;
2. Acetodiphosphonic acids and salts thereof—note German Pat. No. 2,115,427;
3. Lignins, lignosulphonate, starch, sodium mannosinate, agar-agar, polyelectrolytes which contain the group



65 in which R is nitrile, amide, carboxyl or carboxyalkyl and which have a molecular weight of 5,000 to 15,000,000 and water-soluble salts thereof—note U.S. Pat. No. 3,547,817;

4. Amino tri(methyl phosphonic acid) and mono- and poly-phosphonic acids—note U.S. Pat. No. 3,510,436;
5. Polyacrylic acid, polyacrylamide or partially hydrolyzed acrylamide—note U.S. Pat. No. 3,505,238;
6. Aminomethyl phosphonic acid compounds such as those described in U.S. Pat. No. 3,483,133;
7. Derivatives of methanol phosphonic acid or methanol diphosphonic acids such as those described in U.S. Pat. No. 3,532,639; 10
8. The phosphorus-containing polar organic liquids described in U.S. Pat. No. 3,637,790;
9. Leucocyanidin-catechin polymers, carbamates and sodium bisulfate which are described in U.S. Pat. No. 3,518,203; 15
10. Lignosulfonate mixed sugar aldonate polymeric materials such as those described in German Pat. publication No. 2,123,808;
11. Ethylene oxide-propylene oxide polymeric corrosion inhibition compositions containing phosphates, borates, nitrates, silicates and benzoates such as described in German Pat. publication No. 2,054,506; 20
12. 1-hydroxy ethylidene-1,1-diphosphonic acid and water-soluble orthophosphates such as those described in British Pat. No. 1,243,347;
13. A water-dispersible tannin compound and a HCN modified lignosulphate and/or an HCN modified naphthalene sulphonate such as those described in British Pat. No. 1,244,123; 25
14. Silicate materials such as those described in U.S. Pat. No. 3,630,930;
15. Polyfunctional phosphated polyol esters such as those described in U.S. Pat. No. 3,580,855; 30
16. Sulfonated lignites such as those described in U.S. Pat. No. 3,629,105;
17. The polyphosphonic acids such as those described in U.S. Pat. No. 3,619,427; 35
18. Molecularly dehydrated phosphates and phosphonates such as those described in U.S. Pat. No. 3,483,133;
19. Molybdates such as those described in "An Electrochemical Study of Heteropoly Molybdates as Cooling Water Corrosion Inhibitors," A. Weissbuch and C.E. Schell, Paper No. 104 presented at the March, 1972 annual meeting in St. Louis, Mo. of the National Association of Corrosion Engineers (NACE). 40
20. Inorganic Phosphates including orthophosphates.
21. Calcium and magnesium salts such as calcium or magnesium chlorides, sulfates, nitrates and bicarbonates.
22. Cationic organic compounds such as those described in German Pat. publication No. 2,063,208 and German Pat. publication No. 2,063,209. 45
23. Fluidizing polymers such as those described in The Oil And Gas Journal, July 5, 1971, pages 104-5; Plant Engineering, Dec. 1965, pages 133-5; and Chemical Engineering, Dec. 6, 1965, pages 164-8.
24. The scale and corrosion inhibitors such as those described in U.S. Pat. Nos. 3,123,640; 3,123,641; 3,141,905; 3,462,365; 3,477,956; 3,480,083; 3,487,018; 3,518,204; 3,580,855; 3,591,513; 50

3,592,764; 3,592,834; 3,596,766; 3,597,352; 3,617,578; 3,620,974; and 3,644,205.

25. And mixtures of the above materials listed in items 1 through 24.

15 All of the above publications are to be considered as incorporated herein by reference.

In conjunction with the Examples hereinafter set forth, two tests are conducted to determine the effectiveness of the corrosion inhibitors of the present invention in different corrosive media, i.e., ordinary tap water and synthetic cooling tower water.

20 Test 1 is conducted at room temperatures, about 70° F., wherein several coupons of mild steel (S.A.E. 1018) having dimensions of 5 cm × 3.5 cm × 0.32 cm are thoroughly cleaned using a commercially available cleansing powder and rinsed with distilled water and acetone. After the coupons are weighed, they are mounted on brackets and continuously immersed and removed from the corrosion composition, i.e., ordinary tap water, so that the coupons remain immersed in the composition for 60 seconds and then remained out of solution, exposed to air for 60 seconds. This procedure is continued for a definite length of time (in hours) 25 after which the coupons are withdrawn and the corrosion products on the coupons are removed by using a soft brush.

30 The coupons are rinsed with distilled water and acetone and then reweighed. The loss in weight (in milligrams) is then appropriately inserted into the equation:

$$KW/DAT = \text{Corrosion in mills per year}$$

wherein

W = weight loss during tests in milligrams;

D = specific gravity of the metal;

A = exposed surface area in square cm; and

T = time of exposure to solution in hours

K = 3,402

40 in order to determine the corrosion that has taken place expressed in terms of mills of penetration per year (m.p.y.). The corrosion rate of the coupons protected by a corrosion inhibitor can then be compared to the corrosion rate of the unprotected coupons. A decrease in the corrosion rate indicates the effectiveness of the corrosion inhibitor.

50 In tests of this nature where the aqueous corrosive medium is ordinary tap water at room temperature, any corrosion rate less than that corrosion rate of the said medium is desired and rates of less than about 2 to 10 m.p.y. are highly desired and substances that give this range or lower are considered excellent. This does not mean, however, that substances having a corrosion rate of more than about 2 to 10 m.p.y. are not valuable; depending upon the particular conditions a compound or composition having a higher corrosion rate may be used, as in an instance where the equipment will be used, only for a short period of time.

55 60 A cooling water system is constructed on a small scale to approximate conditions for Test 2. From a 5-gallon glass tank containing synthetic cooling water, a hose leads into a 6 in. glass jacket which surrounds a mild steel pipe. A hose leads from the jacket into a glass condenser and then back to the tank. Air is added to the system at the condenser in order to match an actual operation in which air is absorbed by the cooling water.

Steam is passed through the steel pipe which is enclosed by the glass jacket.

Four mild steel coupons are weighed and then mounted in the tank. After exposure the steel pipe is checked visibly for signs of corrosion and the corrosion rate of the coupons is calculated. Synthetic cooling water is prepared to approximate actual cooling water as follows:

|                                              |           |
|----------------------------------------------|-----------|
| Ca <sup>++</sup>                             | 200 ppm   |
| Mg <sup>++</sup>                             | 55 ppm    |
| Na <sup>++</sup>                             | 320 ppm   |
| Cl <sup>-</sup>                              | 600 ppm   |
| SO <sub>4</sub> <sup>-</sup>                 | 500 ppm   |
| HCO <sub>3</sub> <sup>-</sup>                | 58 ppm    |
| Total Dissolved Solids of<br>Distilled Water | 1,733 ppm |

A circulating cooling water system contains a high concentration of inorganic salt or ions much higher than ordinary tap water as can be seen from the formulation for synthetic cooling tower water. Likewise a cooling water system is operated at high temperatures usually 50° C. or higher. Primarily because of these two factors the acceptable corrosion rates in cooling waters is less than about 10 m.p.y. Therefore, corrosion inhibitors having corrosion rates less than about 10 m.p.y. are considered good and commercially acceptable.

The corrosion inhibiting compositions of this invention can be manufactured via a number of methods which will give good protection against corrosion. For example, the SDA either in the form of its acid or salt per se or in combination with the water soluble zinc salt, chromate, dichromate, thiols, 1,2,3-thiazole, silicates, inorganic phosphate, molybdate, tannin, lignin, lignin sulfonate, and calcium and/or magnesium salts, can simply be dissolved by intermixing them into the aqueous corrosive medium. Via another method, they can be dissolved separately in water or another suitable solvent and then intermixed into the aqueous corrosive medium.

Various means are available to insure that the correct proportion of corrosion inhibitor is present in the corrosive medium. For example, a solution containing the said corrosion inhibitor can be metered into the corrosive medium by a drop feeder. Another method is to formulate tablets or briquettes of a "solid" SDA (and other ingredients) and these can then be added to the corrosive medium. The said "solid," after briquetting, can be used in a standard ball feeder so that the "solid" is released slowly into the corrosive medium.

The invention will be further illustrated but is not limited by the following examples:

#### EXAMPLE I

Three separate portions consisting each of 600 ml of aqueous corrosive medium are individually treated with the indicated SDA so that it contains separately 5, 50 and 100 parts per million of SDA. (Where the acid form is used, it is converted to the sodium salt by the addition of sufficient NaOH to maintain the medium at pH 9.0 to 9.5.) Test 1, as described hereinbefore, is conducted using 1018 S.A.E. mild steel coupons measuring 5 cm × 3.5 cm × 0.32 cm. The corrosive medium is a sample of water obtained from the St. Louis County Water Company having a pH from about 9.0 to about

9.5 and a hardness of about 100 to about 110 parts per million as calcium carbonate. Test 1 is conducted according to the procedure hereinbefore outlined for 90 hours. Six hundred ml. of the untreated aqueous corrosive medium is tested as a control. The data are illustrated in Table 1.

Test 1 is also conducted on a commercially available corrosion inhibitor, containing some zinc (about 1 to about 4% by weight) but mostly tetra sodium pyrophosphate (about 50 to about 60% by weight); these data are shown in Table 1.

TABLE I

| Corrosion Rates on Mild Steel (S.A.E. 1018) Coupons<br>5 cm × 3.5 cm × 0.32 cm pH 9.0 to 9.5 of the Corrosive<br>Media |                                                                                                                         |                      |                |                            |
|------------------------------------------------------------------------------------------------------------------------|-------------------------------------------------------------------------------------------------------------------------|----------------------|----------------|----------------------------|
|                                                                                                                        | Corrosion Inhibitor                                                                                                     | Concentration<br>ppm | Time<br>(hrs.) | Corrosion<br>Rate (m.p.y.) |
| 20                                                                                                                     | Corrosion Medium<br>SDA Compound No.                                                                                    |                      | 96             | 25.2                       |
| 25                                                                                                                     |                                                                                                                         |                      |                |                            |
| 30                                                                                                                     | 1                                                                                                                       | 5                    | 96             | 8.9                        |
|                                                                                                                        | 1                                                                                                                       | 50                   | 96             | 5.3                        |
|                                                                                                                        | 1                                                                                                                       | 100                  | 96             | 3.7                        |
|                                                                                                                        | 6                                                                                                                       | 5                    | 96             | 10.2                       |
|                                                                                                                        | 6                                                                                                                       | 50                   | 96             | 8.1                        |
|                                                                                                                        | 6                                                                                                                       | 100                  | 96             | 4.9                        |
| 35                                                                                                                     | 9                                                                                                                       | 5                    | 96             | 6.7                        |
|                                                                                                                        | 9                                                                                                                       | 50                   | 96             | 4.1                        |
|                                                                                                                        | 9                                                                                                                       | 100                  | 96             | 3.8                        |
|                                                                                                                        | 12                                                                                                                      | 5                    | 96             | 9.8                        |
|                                                                                                                        | 12                                                                                                                      | 50                   | 96             | 6.2                        |
|                                                                                                                        | 12                                                                                                                      | 100                  | 96             | 5.1                        |
| 40                                                                                                                     | 16                                                                                                                      | 5                    | 96             | 10.9                       |
|                                                                                                                        | 16                                                                                                                      | 50                   | 96             | 5.9                        |
|                                                                                                                        | 16                                                                                                                      | 100                  | 96             | 3.8                        |
|                                                                                                                        | 18                                                                                                                      | 5                    | 96             | 9.9                        |
|                                                                                                                        | 18                                                                                                                      | 50                   | 96             | 5.2                        |
|                                                                                                                        | 18                                                                                                                      | 100                  | 96             | 3.6                        |
| 45                                                                                                                     | 20                                                                                                                      | 5                    | 96             | 10.4                       |
|                                                                                                                        | 20                                                                                                                      | 50                   | 96             | 5.0                        |
|                                                                                                                        | 20                                                                                                                      | 100                  | 96             | 3.1                        |
|                                                                                                                        | 23                                                                                                                      | 5                    | 96             | 8.7                        |
|                                                                                                                        | 23                                                                                                                      | 50                   | 96             | 5.3                        |
| 50                                                                                                                     | 23                                                                                                                      | 100                  | 96             | 3.6                        |
|                                                                                                                        | Corrosion Medium<br>Zinc - Tetra Sodium<br>Pyrophosphate (Zinc 1% to<br>4%, tetra sodium pyro-<br>phosphate 40% to 60%) | 5                    | 96             | 29.6                       |
|                                                                                                                        |                                                                                                                         | 50                   | 96             | 15                         |
|                                                                                                                        |                                                                                                                         | 100                  | 96             | 6.8                        |
|                                                                                                                        |                                                                                                                         |                      |                | 4.1                        |

The data in Table 1 show that the SDA are an effective corrosion inhibitor. Table 1 shows that these SDA are at least as good as and in some cases superior to the commercially available zinc tetra sodium pyrophosphate inhibitor. As pointed out before, substances that reduce the corrosion rates of mild steel to less than about 10 m.p.y. in ordinary tap water are considered excellent. Therefore, it can readily be appreciated that the SDA of the present invention are effective corrosion inhibitors.

#### EXAMPLE II

Test 2, as described hereinbefore, is conducted to determine the effectiveness of the indicated SDA (Ex-

ample I) as a corrosion inhibitor in cooling water. Example I solutions are individually added to the five gallon tank containing about 16,000 ml. of synthetic cooling tower water (having a flow rate of 2,750 ml./min.), as set forth above, so that said water contains 5, 50 and 100 parts per million of the SDA. The temperature of the synthetic cooling water is 50° C. Mild steel coupons (ASTM A-285) measuring 2.5 cm × 5 cm × .6 cm are cleaned with a commercially available cleansing powder and weighed. They are then mounted on brackets in the five gallon tank. After exposure, they are reweighed and their corrosion rates are calculated.

A blank solution containing no SDA is used as a control to determine the corrosion rates of mild steel coupons in untreated synthetic cooling tower water.

The data show that the SDA corrosion inhibitors at greater than 50 ppm reduce the corrosion rate to less than 10 m.p.y. (the control corrosion medium is about 24.6 m.p.y.), which is the generally acceptable rate for a corrosion inhibitor.

A visual inspection of the mild steel pipe through which the steam passes and which is cooled by the synthetic cooling water treated with SDA shows a very minute amount of corrosion, another indication of the effectiveness of the novel compound of the present invention.

A commercial corrosion inhibitor containing 2 to 4 percent by weight of zinc and 40 to 60 percent by weight of tetra sodium pyrophosphate, is used to treat the synthetic cooling water and is tested in the same manner as Example II. The corrosion rates of the coupons are more than 10 m.p.y. and a significant amount of corrosion forms on the mild steel pipe through which the steam passes.

It can readily be appreciated that these SDA are good corrosion inhibitors when used in cooling waters and especially when used in heat-exchanging systems.

### EXAMPLE III

Example I (above) is repeated with the exception that in addition to the SDA (5, 500 and 100 ppm) corrosion inhibitor, there is added sufficient amounts of zinc sulfate in order to provide respectively 5, 50 and 100 ppm of zinc ion in the corrosion medium. This corrosion inhibition composition, i.e., the indicated SDA plus the zinc sulfate, shows that at all three concentrations (i.e., 5, 50 and 100 ppm of each) the corrosion rates are substantially less than the rates using the corrosion medium without this mixture and is on the average 25 percent less than those rates obtained using only the SDA per se.

### EXAMPLE IV

Example I (above) is repeated with the exception that in addition to the SDA (5, 50 and 100 ppm) corrosion inhibitor, there is added respectively 5, 50 and 100 ppm sodium dichromate to the corrosion medium. This corrosion inhibition composition, i.e., the indicated SDA plus the sodium dichromate, shows that at all three concentrations (i.e., 5, 50 and 100 ppm of each), the corrosion rate is less than the rate using the corrosion medium without this mixture and is on the average about 11 to 20 percent less than those rates obtained using only the SDA per se.

### EXAMPLE V

A series of separate and individual corrosion inhibitors consisting of a mixture of the indicated SDA (60% by weight), zinc sulfate (20 percent by weight) and sodium dichromate (20% by weight) are prepared. Example I (above) is then repeated utilizing the above mixture. The resultant data shows that the corrosion rates using this mixture are substantially less than the rates using the corrosion medium without this mixture and is on the average about 30 to 40 percent less than those rates obtained using only the SDA per se.

### EXAMPLE VI

15 The corrosion inhibitors are described in the above Examples I, III, IV and V are separately and individually tested in boiler water for their separate corrosive inhibiting effect on red brass and mild steel. The boiler water contains approximately 30-60 parts per million phosphate and approximately 30-60 parts per million sulfate having a pH of about 14. The corrosive tests are carried out at a temperature of 314° C. at 1,500 psig and with a 50 parts per million of the respective corrosion inhibitor. In each test, approximately 1 liter of boiler blow-down water is charged into a 2 liter bomb and 1 ml. of a stock solution is added to give approximately 50 parts per million of the corrosion inhibitor. Duplicate coupons of mild steel and red brass measuring 5 cm × 3.5 cm × 0.32 cm are scrubbed with a commercially available cleansing powder and weighed. The coupons are then mounted on insulated brackets so that two coupons are in the liquid phase and two coupons are in the vapor phase. After sealing 25 the bomb, the cycle of pumping down with a vacuum pump and filling with nitrogen is repeated four times. The time of the tests are taken to be roughly from the time the temperature reached 150° C. after starting to heat till it again reached this temperature after turning 30 off the heat.

The results of these tests show that at temperatures above 300° C. the respective corrosion inhibitors significantly reduces the corrosion rates of both red brass and mild steel either completely immersed in the cooling waters or in contact with the vapors of a cooling water system containing the complex. It also demonstrates the stability of the corrosion inhibitors of the present invention at elevated temperatures, over 300° C., for extended periods of time.

45 50 In each of the following examples, the indicated SDA and zinc compound are added to the aqueous corrosive medium so that 50 parts per million of each is present.

### EXAMPLE VII

| Ingredients              | Parts  |
|--------------------------|--------|
| Aqueous corrosive medium | 75,000 |
| SDA Compound No. 1       | 2      |
| Zinc sulfate             | 2      |

### EXAMPLE VIII

| Ingredients              | Parts  |
|--------------------------|--------|
| Aqueous corrosive medium | 80,000 |
| SDA Compound No. 6       | 2.6    |
| Zinc sulfate             | 2.6    |

## EXAMPLE IX

| Ingredients              | Parts  |
|--------------------------|--------|
| Aqueous corrosive medium | 90,000 |
| SDA Compound No. 9       | 2.3    |
| Zinc sulfate             | 2.3    |

## EXAMPLE X

| Ingredients              | Parts  |
|--------------------------|--------|
| Aqueous corrosive medium | 90,000 |
| SDA Compound No. 12      | 2.3    |
| Zinc sulfate             | 2.3    |

## EXAMPLE XI

| Ingredients              | Parts  |
|--------------------------|--------|
| Aqueous corrosive medium | 90,000 |
| SDA Compound No. 16      | 2.3    |
| Zinc sulfate             | 2.3    |

## EXAMPLE XII

| Ingredients              | Parts  |
|--------------------------|--------|
| Aqueous corrosive medium | 65,000 |
| SDA Compound No. 18      | 1.6    |
| Zinc sulfate             | 1.6    |

## EXAMPLE XIII

| Ingredients              | Parts  |
|--------------------------|--------|
| Aqueous corrosive medium | 11,000 |
| SDA Compound No. 20      | 2.7    |
| Zinc sulfate             | 2.7    |

## EXAMPLE XIV

| Ingredients              | Parts   |
|--------------------------|---------|
| Aqueous corrosive medium | 100,000 |
| SDA Compound No. 23      | 2.5     |
| Zinc sulfate             | 2.5     |

(The sodium salts of the above Compound Nos. 1, 6, 9, 12, 16, 18, 20 and 23 are used in place of the acid forms.) Tests 1 and 2 are conducted on each of the above-treated aqueous corrosive media. The corrosion rates in all instances are lower than the untreated corrosive media. These Examples are repeated with the exception that the zinc salt used is zinc chloride (in one repeat) and zinc acetate (in another repeat). Similar results are obtained in both cases as compared to the results obtained using zinc sulfate.

## EXAMPLE XV

25 A compressed ball of a standard weight and dimension is prepared containing the following ingredients in the quantities noted.

|                                 |    |
|---------------------------------|----|
| SDA Compound No. 1              | 34 |
| Lignosulfite binder (bindarene) | 8  |
| Zinc sulfate                    | 16 |
| Inert Ingredients               | 42 |

35 The above composition after briquetting is found suitable for mechanically measured addition in water treatment wherein a ball feeder is employed.

## EXAMPLE XVI

Example I (above) is repeated with the exception 40 that copper coupons are used instead of mild steel coupons and sufficient amounts of 1,2,3-benzotriazole to provide 1, 5 and 10 ppm thereof in the corrosive media is used in addition to the SDA. Example XVI is repeated again but without the benzotriazole material. 45 The data shows that when copper coupons are used and the corrosive media contains the indicated SDA, the corrosion rates are less than when the corrosion media does not contain said SDA. The data further show that 50 use of the benzotriazole with the SDA further reduces the corrosion rate.

It is also within the scope of the present invention to utilize silicates, particularly inorganic silicates, in combination with the SDA. It is known that silicates are effective corrosion inhibitors as exemplified by "Encyclopedia of Chemical Technology," Kirk-Othmer, 1961 by The Interscience Encyclopedia, Inc. New York - Volume 4, pages 487-529, and Volume 12, pages 268-360; this subject matter is to be considered 55 as incorporated herein by reference. (These silicates can be used in the same concentration as the water-soluble zinc salts heretofore mentioned.)

It is found in the repeat of the above Example I that 60 the use of a combination of the indicated SDA and a liquid (sodium) silicate (having a 3.22:1 ratio of  $\text{SiO}_2$  to soda) effected a lower corrosion rate than either the SDA per se or the silicate per se when used separately.

Thus, it may be seen that this invention relates to the indicated SDA falling within Formula I above as corrosion inhibitors. We do not intend to be limited to any compounds, composition, or methods disclosed herein for illustrative purposes. Our invention may be otherwise practiced and embodied within the scope of the following claims.

What is claimed is:

1. A composition useful for inhibiting the corrosion of metals in a water system consisting essentially of from about 10 percent to about 80 percent by weight of a water-soluble zinc salt and from about 20 to 90 percent by weight of a substituted diamine having the general formula



wherein (a) R<sub>1</sub> and R<sub>2</sub> are alike or unlike and are selected from the group consisting of hydrogen, metal ions, amine ions or any cation which will provide sufficient solubility in said aqueous system, mixtures thereof; (b) R<sub>3</sub> and R<sub>4</sub> are alike or unlike and are each independently an alkylene group containing from about two to about five carbon atoms; (c) n is an integer having a value of from about 0 to about 10; (d) X and Y are each alike or unlike and are selected from the group consisting of hydrogen, aromatic and alkyl; and (e) Z is a hydrocarbon group containing from two to 15 carbon atoms.

2. The composition as set forth in claim 1 wherein X and Y both are hydrogen.

3. The composition as set forth in claim 2 wherein R<sub>1</sub> and R<sub>2</sub> are each hydrogen.

4. The composition as set forth in claim 2 wherein R<sub>1</sub> and R<sub>2</sub> are each a cation selected from the group consisting of alkali metals, ammonia, zinc, and mixtures thereof.

5. The composition as set forth in claim 4 wherein the water-soluble zinc salt is zinc sulfate and at least one of R<sub>1</sub> and R<sub>2</sub> is sodium.

6. The composition as set forth in claim 1 and additionally containing a water-soluble hexavalent compound of chromium.

7. A composition useful for inhibiting the corrosion of metals in a water system which contains cuprous metals consisting essentially of (1) from about 20 percent to about 90 percent by weight of a substituted diamine having the general formula



wherein (a) R<sub>1</sub> and R<sub>2</sub> are alike or unlike and are selected from the group consisting of hydrogen, metal ions or any cation which will provide sufficient solubility in said aqueous system and amine ions (as defined in

the specification) and mixtures thereof; (b) R<sub>3</sub> and R<sub>4</sub> are alike or unlike and are each an alkylene group containing from about two to five carbon atoms; (c) X and Y are each alike or unlike and are selected from the group consisting of hydrogen aromatic and alkyl; (d) Z is a hydrocarbon group containing from two to 15 carbon atoms, and (e) n has a value of from 1 through 10; (2) from about 1 percent to about 10 percent by weight of a compound selected from the group consisting of 1,2,3-triazoles, thiols of thiazoles, thiols of oxazoles, thiols of imidazoles, and mixtures thereof, and (3) up to about 79 percent by weight of a water-soluble zinc salt.

8. The composition as set forth in claim 7 and additionally containing a water-soluble hexavalent compound of chromium.

9. A composition useful for inhibiting the corrosion of metals in a water system consisting essentially of from about 2 to about 80 percent by weight of a silicate and from about 20 percent to about 98 percent by weight of a substituted diamine having the general formula



wherein (a) R<sub>1</sub> and R<sub>2</sub> are alike or unlike and are selected from the group consisting of hydrogen, metal ions, or any cation which will provide sufficient solubility in said aqueous system and mixtures thereof; (b) R<sub>3</sub> and R<sub>4</sub> are alike or unlike and are each independently an alkylene group containing from about two to about five carbon atoms; (c) n is an integer having a value of from about 0 to about 10; (d) X and Y are each alike or unlike and are selected from the group consisting of hydrogen, aromatic and alkyl; and (e) Z is a hydrocarbon group containing from two to 15 carbon atoms.

10. The composition as set forth in claim 1 wherein the substituted diamine has the formula



11. The composition as set forth in claim 1 wherein the substituted diamine has the formula



12. The composition as set forth in claim 1 wherein the substituted diamine has the formula



13. The composition as set forth in claim 1 wherein the substituted diamine has the formula



14. The composition as set forth in claim 1 wherein the substituted diamine has the formula



15. The composition as set forth in claim 1 wherein the substituted diamine has the formula



16. The composition as set forth in claim 1 wherein the substituted diamine has the formula



17. The composition as set forth in claim 1 wherein the substituted diamine has the formula



18. The composition as set forth in claim 1 wherein the substituted diamine has the formula



19. The composition as set forth in claim 1 wherein the substituted diamine has the formula



**20.** The composition as set forth in claim 1 wherein the substituted diamine has the formula



21. The composition as set forth in claim 1 wherein the substituted diamine has the formula



22. The composition as set forth in claim 1 wherein  
30 the substituted diamine has the formula



23. The composition as set forth in claim 1 wherein  
40 the substituted diamine has the formula



24. The composition as set forth in claim 1 wherein the substituted diamine has the formula



25. The method of inhibiting the corrosion of metals in a water system comprising maintaining in the water of said system at least 3 parts per million of a substituted diamine having the general formula



wherein (a)  $R_1$  and  $R_2$  are alike or unlike and are selected from the group consisting of hydrogen, metal ions or any cation which will provide sufficient solubility in said aqueous system and amine ions (as defined in the specification) and mixtures thereof; (b)  $R_3$  and  $R_4$  are alike or unlike and are each an alkylene group containing from about two to five carbon atoms; (c) X and Y are each alike or unlike and are selected from the group consisting of hydrogen, aromatic and alkyl; (d) Z is a hydrocarbon group containing from two to 15 carbon atoms, and (e)  $n$  has a value of from 1 through 10.

26. The method as set forth in claim 25 wherein X and Y both are hydrogen.

27. The method as set forth in claim 26 wherein  $R_1$  and  $R_2$  are each hydrogen.

28. The method as set forth in claim 26 wherein  $R_1$  and  $R_2$  are each a cation selected from the group consisting of alkali metals, ammonia, zinc, and mixtures thereof.

29. The method as set forth in claim 25 and additionally containing in said system a water-soluble hexavalent compound of chromium.

30. The method as set forth in claim 25 and additionally containing in said system a water-soluble zinc salt.

5 10

31. The method as set forth in claim 25 and additionally containing in said system a water-soluble hexavalent compound of chromium and a water-soluble zinc salt.

32. The method as set forth in claim 25 wherein said system contains cuprous metals and the water system additionally contains a compound selected from the group consisting of 1,2,3-triazoles, thiols of thiazoles, thiols of oxazoles, thiols of imidazoles, and mixtures thereof.

33. The method as set forth in claim 32 wherein the water system additionally contains a water-soluble zinc salt.

34. A method of inhibiting metal corrosion in a water system containing metals comprising maintaining in the water of said system (a) from about 3 to about 100 ppm of a substituted diamine having the formula



or its water-soluble salts and (b) up to about 100 ppm zinc ion derived from water-soluble zinc salts.

\* \* \* \* \*